# EUROPEAN PATENT SPECIFICATION

(11) **EP 2 636 725 B1**
(45) Date of publication and mention of the grant of the patent: **08.05.2019**
(21) Application number: 13157940.1
(22) Date of filing: 06.03.2013
(51) Int. Cl.: C10M 171/02, C10N 30/06, C10N 40/25

(54) **Lubricating oil composition for automobile engine lubrication**
Schmierölzusammensetzung für die Schmierung eines Automobilmotors
Composition d'huile lubrifiante pour la lubrification d'un moteur automobile

(30) Priority: 08.03.2012 JP 2012051849
(43) Date of publication of application: 11.09.2013
(73) Proprietor: Chevron Japan Ltd., Tokyo 101-0041 (JP)
(72) Inventor: Hiroki, Andoh, Omaezaki-shi, Shizuoka (JP); Nakazato, Morikuni, Omaezaki-shi, Shizuoka (JP)
(74) Representative: Haseltine Lake LLP

(56) References cited:
- WO-A1-2011/115265
- US-A- 5 863 873
- US-A1- 2009 163 393
- TAYLOR ET AL: "Improved fuel efficiency by lubricant design: A review", PROCEEDINGS OF THE INSTITUTION OF MECHANICAL ENGINEERS, PART J.JOURNAL OF ENGINEERING TRIBOLOGY, MECHANICAL ENGINEERING PUBLICATIONS, BURY ST. EDMUNDS, GB, vol. 214, no. 1, 1 January 2000 (2000-01-01), pages 1-15, XP009169924, ISSN: 1350-6501

## Description

This application claims priority to Japanese Patent Application number JP 2012-51849 which was filed on March 8, 2012.

### Field of Invention

The present invention relates to an excellent fuel-efficient, low-viscosity lubricating oil composition for an automobile engine, and in particular, relates to a lubricating oil composition for automobile engine lubrication that, while being an excellent fuel-efficient, low-viscosity lubricating oil composition for engine lubrication, also shows high wear resistance. The present invention relates to a low-viscosity lubricating oil composition that is particularly suitable for lubricating a motorcycle four-cycle gasoline engine or a diesel engine having an exhaust gas after-treatment device.

### Background of Invention

There is an increasing demand for improved fuel efficiency in automobiles. Therefore, there is a need for an excellent fuel-efficient, low-viscosity engine oil as the lubricating oil composition (engine oil) that is used to lubricate the engine of a gasoline engine vehicle or a diesel engine vehicle. For instance, engine oils that have an SAE viscosity grade of 5W20 and a high-temperature high-shear viscosity (value measured at 150°C when the shear velocity or shear rate is 10⁶ s⁻¹) of 2.6 mPa·s are already being used for practical purposes as fuel-efficient lubricating oil compositions for gasoline engines in four-wheel drive vehicles.

However, by means of four-cycle gasoline engines for motorcycles, the engine oil is also used to lubricate the transmission system and there is a chance that wear of the energy-transmission devices, such as the transmission gears, will increase (wear resistance will decrease) as a result of a reduction in viscosity of the engine oil. Taking this point into consideration, JASO T903-2006 stipulates that the engine oils for motorcycle four-cycle gasoline engines have a high-temperature, high-shear (10⁶s⁻¹) viscosity of 2.9 mPa·s or greater. Nevertheless, such a high high-temperature, high-shear viscosity can hardly been expected of the SAE5W20 engine oils known today and therefore, the engine oils used today in motorcycle four-cycle gasoline engines are all low-viscosity engine oils of SAEI viscosity grade 10W30, 5W30, or 0W30.

On the other hand, taking into consideration the need for wear resistance in engine oils, ACEA C1-08 and C2-08, which are the European standards for engine oils appropriate for lubrication of diesel engine vehicles having diesel particulate filters, set the lower limit of high-temperature, high-shear (10⁶s⁻¹) viscosity of engine oils at 2.9 mPa·s and, in order to limit evaporation loss of engine oils, the upper limit of NOACK evaporation loss at 13%.

Patent Document JP (Kokai) 6-306384 describes a fuel-efficient lubricating oil for an internal combustion engine wherein a predetermined amount of an organic molybdenum compound is added to a mineral oil base oil having a dynamic viscosity at 100°C of 3 to 5 cSt, a viscosity index of 135 or higher, and a paraffin to total carbon ratio (%Cp) of 90% or higher.

Patent Document JP (Kohyo) 2003-505533 describes a lubricating oil composition that, as a molybdenum additive-free, fuel-efficient, low-volatility lubricating oil composition having a NOACK volatility of 15 wt% or less, contains a predetermined amount of a calcium detergent and a predetermined amount of an oil-soluble organic wear-improving agent, as well as a base oil comprising at least 50 wt% of mineral oil; has a dynamic viscosity at 100°C of 4.0 to 5.5 mm²/s; contains 95 wt% or more of saturated product and 25 wt% or less of naphthenes; has a viscosity index of at least 120; and has an NOACK volatility of 15.5 wt% or less.

Patent Document JP (Kokai) 2000-87070 describes an excellent fuel-efficient motorcycle four-cycle engine composition having an oil consumption-lowering effect that contains a hydrocarbon lubricating oil base oil having a dynamic viscosity at 100°C of 3 to 10 mm²/s and a viscosity index of 120 or higher, or a mixed base oil containing at least 15 mass% of this base oil, a zinc dialkyl dithiophosphate, a metal detergent, an ash-free dispersant, a wear regulator, and a viscosity index-improving agent that brings dynamic viscosity at 100°C of this composition to 9.3 to 16.5 mm²/s. Specifically, it describes a motorcycle four-cycle engine composition having an SAE viscosity grade of 10W30 or 10W40.

US2009/163393 A1 discloses lubricating oil for high performance engines comprising a Group III base oil and a combination of ester base stocks.

### Summary of Invention

Improving engine structure is of course important as a method for improving fuel efficiency of automobile engines, but it is also known that lowering viscosity of lubricating oils is effective in improving fuel efficiency. Therefore, as previously mentioned, engine oils having an SAE viscosity grade of 5W20 and a high-temperature, high-shear (10⁶s⁻¹) viscosity of 2.6 mPa·s are already being used as fuel-efficient gasoline engine oils for four-wheel drive vehicles. Nevertheless, fuel-efficient gasoline engine oils for four-wheel drive vehicles having an SAE viscosity grade of 5W20 cannot be expected to have a high-temperature, high-shear viscosity that is as high as 2.6 mPa·s and therefore, there is a problem in that when used as the engine oil of a motorcycle four-cycle gasoline engine that uses engine oil for lubrication of the transmission system, there is a problem in that wear resistance is insufficient.

The inventors completed the present invention upon discovering that it is possible to produce a lubricating oil composition that has an SAE viscosity grade of 5W20 and yet a viscosity index within a range of 140 to 230, a high-shear (10⁶s⁻¹) viscosity at 150°C of 2.9 mPa·s or higher, a NOACK evaporation loss of 13% or less, and excellent wear resistance by using a base oil such as has been recently supplied to the market and is primarily isoparaffin, has an ultrahigh viscosity index wherein the viscosity index is within a range of approximately 133 to 160, and is obtained by hydrogenation and isomerization of a slack wax or a synthetic wax produced by the Fischer-Tropsch method and distillation and dewaxing treatment, and by optimizing the combination of additive components added to the base oil and the amount of each lubricant component. Note that lubricating oil compositions of SAE viscosity grade 5W20 are already known to have excellent fuel efficiency because they have a relatively low dynamic viscosity under temperature conditions of both low temperatures and high temperatures.

Consequently, the present invention is a lubricating oil composition for automobile engine lubrication, which is a lubricating oil composition comprising a base oil and the following additive components and having an SAE viscosity grade of 5W20, wherein the viscosity index is within a range of 140 to 230, the high-shear viscosity at 150°C is 2.9 mPa·s or higher, and the NOACK evaporation loss is 13% or less, further comprising:
a) a nitrogen-containing ash-free dispersant at 0.01 to 0.3 mass% in terms of the nitrogen content,
b) an alkaline earth metal-containing detergent at 0.08 to 0.4 mass% in terms of alkaline earth metal content,
c) a phosphorus-containing anti-wear agent at 0.05 to 0.12 wt% in terms of phosphorus content,
d) an antioxidant selected from the group consisting of amine compounds, phenol compounds, and molybdenum compounds at 0.1 to 7 mass%,
e) a viscosity index-improving agent at 0.5 to 20 mass%, and further wherein the amount of each additive component is the mass% in terms of the total amount of lubricating oil composition;
wherein the Noack evaporation loss is determined by ASTM D5800; and
wherein the phrase "high-shear viscosity" refers to the measured value (shear viscosity) when the shear speed or shear rate is 10⁶s⁻¹, and
wherein the base oil is:
a base oil comprising as a base oil component at least 80 mass% of a mineral oil base oil having a kinematic viscosity at 100°C that is within a range of 2 to 9 mm²/s and a viscosity index of 133 to 160; or
a base oil having a viscosity index of 133 to 160 that is obtained by hydrogenation and isomerization of either a slack wax or a synthetic wax produced by the Fischer-Tropsch method and then distillation and dewaxing treatment.

It should be noted that the phrase "lubricating oil composition having an SAE viscosity grade of 5W20 of the present invention" refers to a lubricating oil composition that satisfies the viscosity property of "5W20" described in "SAE viscosity grades for engine oils" of the American Petroleum Institute (revised in 2007). Moreover, the phrase "high-shear viscosity" refers to the measured value (shear viscosity) when the shear speed or shear rate is 10⁶s⁻¹.

The present invention also is a method for lubricating a motorcycle four-cycle gasoline engine or a diesel engine having an exhaust gas after-treatment device.

### Detailed Description of the Invention

The lubricating oil composition for lubricating an automobile engine provided by the present invention is a lubricating oil composition having an SAE viscosity grade that is low at 5W20, while having a high-temperature, high-shear viscosity of 2.9 mPa·s or higher, and shows excellent fuel efficiency and wear resistance. The lubricating oil compositor of the present invention therefore is an excellent fuel-efficient, wear-resistant lubricating oil that is particularly suitable for lubricating a motorcycle four-cycle gasoline engine or a diesel engine having an exhaust gas after-treatment device.

The following are preferred modes of the lubricating oil composition for lubricating an automobile engine of the present invention.
(1) Kinematic viscosity at 100°C is within a range of 8.5 mm²/s or greater, but less than 9.3 mm²/s.
(2) The base oil comprises as a base oil component at least 80 mass% of a mineral oil base oil having a kinematic viscosity at 100°C that is within a range of 2 to 9 mm²/s (particularly preferably 4.5 to 9 mm²/s, further preferably 5 to 8.5 mm²/s) and a viscosity index of 133 to 160.
(3) The base oil is a mineral oil having a kinematic viscosity at 100°C that is within a range of 2 to 9 mm²/s (particularly preferably 4.5 to 9 mm²/s, further preferably 5 to 8.5 mm²/s) and a viscosity index of 133 to 160.
(4) The base oil is a base oil having a viscosity index of 133 to 160 that is obtained by hydrogenation and isomerization of either a slack wax or a synthetic wax produced by the Fischer-Tropsch method and then distillation and dewaxing treatment.
(5) The lubricating oil comprises two or more base oil components having different viscosities, but both having a viscosity index of 130 or higher.
(6) The viscosity index-improving agent is a polymethacrylate polymer having a shear stability index (SSI, as defined by ASTM D6022) of 30 or less.
(7) An organic sulfur compound is further added as an additive component.
(8) The nitrogen-containing ash-free dispersant is a succinimide compound having a bis structure.
(9) The alkaline earth metal-containing component is a perbasic calcium-containing compound selected from the group consisting of perbasic calcium sulfonate and perbasic calcium phenate.
(10) The phosphorus-containing anti-wear agent is a phosphorus-containing compound selected from zinc dihydrocarbyl dithiophosphate and zinc dihydrocarbyl phosphate.
(11) The viscosity index-improving agent is a polymethacrylate viscosity index-improving agent.
(12) The lubricating oil composition is for lubrication of a motorcycle four-cycle gasoline engine.
(13) The lubricating oil composition is for lubricating the engine of a diesel engine vehicle having an exhaust gas post-purification device.

The base oil and additive components that are contained in the lubricating oil composition of the present invention will now be described.

### Base oil

Taking into consideration economics, the base oil of the lubricating oil composition of the present invention is preferably a mineral oil. It can also be a mixture of a relatively large amount (at least 50 mass%) of a mineral oil and a relatively small amount (less than 50 mass%) of a synthetic oil.

Preferably the base oil used in the lubricating oil composition of the present invention is a base oil that is primarily an isoparaffin and has a kinematic viscosity at 100°C of 2 to 9 mm²/s, a saturated component content of 95 mass% or higher (particularly 98 mass% or higher), and a viscosity index of 133 or higher (particularly 135 or higher, further 145 or higher). A base oil having such properties and composition can be used alone, or a combination of two or more types can be used. Moreover, it is also possible to use a mixture of a base oil having such properties and composition and a relatively small amount of a base oil having other properties and composition. Preferably the base oil composition after mixing will still have the above-mentioned properties and composition.

The base oil having the above-mentioned properties and composition preferably has an evaporation loss (ASTM D5800) of 16% or less (particularly 15% or less, further 13% or less). When evaporation loss of the base oil is high, oil consumption with long-term use of an engine oil that uses this base oil (lubricating oil composition) under high temperatures increases, and the rise in viscosity increases. This leads to a reduction in fuel efficiency.

There are no particular restrictions to the type of base oil showing the above-mentioned properties and composition, but when the base oil is a mineral oil, preferably it is a high-viscosity index base oil (base oil having a viscosity index between 133 and 160) the primary component of which is isoparaffin obtained by subjecting the slack wax that is the by-product of dewaxing during the production of mineral oil lubricating base oils, or synthetic wax synthesized using natural gas as the starting material (by the Fischer-Tropsche method), to hydrogenation and isomerization and then distillation and dewaxing. Such a high viscosity index base oil has a relatively high dynamic viscosity at 100°C, but has good low-temperature viscosity properties and therefore, can have a reduced evaporation loss and is ideal as the base oil of the lubricating oil composition of the present invention.

It should be noted that, as described above, the high-viscosity-index base oil, which is the above-mentioned mineral oil, can be used together with a synthetic oil. Preferably the synthetic oil has the above-mentioned properties and composition. The preferred synthetic oil can be selected from a variety of conventional synthetic oils, and examples of such synthetic oils are various esters, alkylbenzenes, and polyalphaolefins (PAO). Poly-alphaolefins (PAOs) are particularly preferred.

### Nitrogen-containing ash-free dispersant

The lubricating oil composition of the present invention comprises a nitrogen-containing ash-free dispersant (component a) in an amount within a range of 0.01 to 0.3 mass% in terms of the nitrogen content. Preferably the mass-average molecular weight of the nitrogen-containing ash-free dispersant is within a range of 4,500 to 20,000. The phrase "mass-average molecular weight" used in the present specification is the molecular weight determined by GPC analysis with polystyrene as the standard substance.

Typical examples of the nitrogen-containing ash-free dispersant used in the lubricating oil composition of the present invention are alkenyl and alkyl succinimides derived from polyolefins and derivatives of these succinimides. The amount added is within a range of 0.01 to 0.3 mass% in terms of the nitrogen content based on the total mass of the lubricating oil composition. Typical succinimides are obtained by reacting a succinic anhydride substituted by alkenyl or alkyl groups and having a high molecular weight and a polyalkylene polyamine containing an average of four to ten (preferably five to seven) nitrogen atoms per molecule. The succinimide anhydride that is substituted by alkenyl or alkyl groups and has a high molecular weight is preferably a polyolefin having a number-average molecular weight of approximately 900 to 5,000, particularly polybutene.

In many cases, chlorination by chlorine is used during the step for obtaining a polybutenyl succinimide by reacting polybutene and maleic anhydride. However, although reactivity is good by this method, it has the effect of a large amount of chlorine (for instance, approximately 2,000 ppm) remaining in the succinimide final product. On the other hand, when thermal reaction that does not use chlorine is employed, the residual chlorine contained in the final product can be kept to a very low level (for instance, 30 ppm or less). Moreover, when polybutene (at least approximately 50% of which is a methylvinylidene structure) having a high reactivity in comparison to conventional polybutene (that is primarily β-olefin in structure) is used, there is an advantage in that reactivity is increased, even by the thermal reaction method. The amount of unreacted polybutene in the dispersant decreases as the reactivity increases and therefore, it is possible to obtain a dispersant having a high effective component (succinimide) concentration. Consequently, preferably the succinimide that is used is produced by obtaining a polybutenyl succinimide anhydride by thermal reaction using highly reactive polybutene and then reacting this polybutenyl succinic anhydride with a polyalkylene polyamine having an average of four to ten nitrogen atoms (per one molecule). This succinimide can be further reacted with boric acid or an alcohol, aldehyde, ketone, alkyl phenol, cyclic carbonate, organic acid, and the like and used as a so-called modified succinimide. In particular, a boric acid-containing alkenyl (or alkyl) succinimide obtained by reaction with boric acid or a boron compound can be used in order to efficiently increase thermal and oxidation stability. Examples of this succinimide are mono-types, bis-types, and poly-types in accordance with the number of imide structures per molecule, but the bis-type or poly-type is preferred as the succinimide used for the purpose of the present invention.

Examples of other nitrogen-containing ash-free dispersants are polymeric succinimide dispersants derived from ethylene-α-olefin copolymer (having a molecular weight of 1,000 to 15,000, for instance) and alkenyl benzylamine ash-free dispersants.

According to the lubricating oil composition of the present invention, Nitrogen-containing dispersion-type viscosity index improvers can also be used in place of the nitrogen-containing ash-free dispersant. A nitrogen-containing olefin polymer or a nitrogen-containing polymethacrylate having a mass-average molecular weight of 90,000 or greater (in terms of polystyrene molecular weight by GPC analysis) is used as the nitrogen-containing dispersion-type viscosity index-improving agent. Taking thermal stability into consideration, the former nitrogen-containing olefin copolymer is effective.

The lubricating oil composition of the present invention contains a nitrogen-containing ash-free dispersant and/or nitrogen-containing dispersion-type viscosity index-improving agent as an active ingredient. These can also be used in combination with another ash-free dispersant, such as an alkenyl succinic acid ester ash-free dispersant.

### Metal-containing detergent

The lubricating oil composition of the present invention contains, as a metal-containing detergent, an alkaline earth metal-containing detergent (component (b)) in an amount within a range of 0.08 to 0.4 mass%. Examples of alkaline earth metals are calcium, barium, and magnesium, but calcium is preferred. Moreover, preferably a sulfonate or phenate of the alkaline earth metal is used as the metal-containing detergent. A combination of a sulfonate of an alkaline earth metal and a phenate of an alkaline earth metal can also be used. It is also possible to use a combination of these metal-containing detergents and a metal-containing detergent such as an alkyl salicylate and/or alkyl carboxylate of an alkaline earth metal (particularly calcium).

Examples of calcium sulfonates are perbasic calcium sulfonate having a total base value of 150 to 500 mgKOH/g and low-basic calcium sulfonate having a total base value of 5 to 60 mgKOH/g. Preferably the perbasic calcium sulfonate is perbasic alkylated calcium benzene sulfonate or alkylated calcium toluene sulfonate having alkyl groups with 10 or more carbon atoms (usually the degree of perbasic conversion is within a range of 5 to 25). On the other hand, preferably the low-basic calcium sulfonate is alkylated calcium benzene sulfonate or alkylated calcium toluene sulfonate having alkyl groups with ten or more carbon atoms and is usually one that is nearly a neutral salt subjected to virtually no perbasic conversion (preferably the degree of perbasic conversion is within a range of 0.1 to 1.5). However, preferably a combination of a perbasic calcium sulfonate and a low-basic calcium sulfonate is used. It should be noted that the sulfonate can be a synthetic sulfonate as described above, or it can be a petroleum sulfonate obtained by sulfonating a lubricating oil fraction of a mineral oil to a calcium salt. Consequently, a petroleum low-basic calcium sulfonate/perbasic calcium sulfonate such as described above is preferred for the purpose of the present invention.

Perbasic sulfurized calcium phenate having a total base value of 120 to 350 mgKOH/g is known as a calcium phenate. A perbasic sulfurized alkyl phenol calcium having alkyl groups with ten or more carbon atoms is preferred.

### Phosphorus-containing anti-wear agent

The lubricating oil composition of the present invention contains a phosphorus-containing anti-wear agent (component c) in an amount within a range of 0.05 to 0.12 mass% in terms of the amount of phosphorus. Preferred phosphorus-containing anti-wear agents are zinc dihydrocarbyl dithiophosphate, zinc dihydrocarbyl monothiophate, and zinc dihydrocarbyl phosphate, which are known as lubricating oil additives that are multiperformance in that they have antioxidant performance and anti-wear performance.

A primary or secondary alkyl group-type zinc dialkyl dithiophosphate is usually used as the zinc dihydrocarbyl dithiophosphate. A zinc dialkyl dithiophosphate having secondary alkyl groups derived from a C₃₋₁₈ secondary alcohol is effective in terms of anti-wear performance. In contrast to this, a zinc dialkyl dithiophosphate having primary alkyl groups derived from a C₃₋₁₈ primary alcohol has a tendency toward being superior in terms of heat resistance and wear-reducing activity. Moreover, a combination of a secondary alkyl group-type zinc dialkyl dithiophosphate and a primary alkyl group-type zinc dialkyl dithiophosphate can be used. Furthermore, it is also possible to use a zinc dialkyl dithiophosphate that is a mixed type of primary and secondary alkyl groups derived from a mixed alcohol of a primary alcohol and a secondary alcohol.

A zinc dialkylaryl dithiophosphate (such as a zinc dialkylaryl dithiophosphate derived from dodecyl phenol) can also be used as the phosphorus-containing anti-wear agent.

Moreover, it is also possible to use a phosphoric acid ester, phosphorus acid ester, or thiophosphoric acid ester as the phosphorus-containing anti-wear agent.

### Anti-oxidant

The lubricating oil composition of the present invention further contains, in an amount that is within a range of 0.1 to 7 mass%, at least one antioxidant (component d) selected from the group consisting of phenol compounds (phenol antioxidants), amine compounds (amine antioxidants), and molybdenum compounds (molybdenum antioxidants).

A hindered phenol compound is generally used as the phenol antioxidant, and a diaryl amine compound is generally used as the amine antioxidant. Hindered phenol antioxidants and diaryl amine antioxidants are both also effective in improving high-temperature detergency. Diaryl amine antioxidants in particular have a base value derived from nitrogen and are effective in improving high-temperature detergency. On the other hand, hindered phenol antioxidants are effective in preventing oxidative degradation by NOₓ.

Examples of hindered phenol antioxidants are 2,6-di-t-butyl-p-cresol, 4,4'-methylenebis(2,6-di-t-butylphenol), 4,4'-methylenebis(6-t-butyl-o-cresol), 4,4'-isoropylidenebis(2,6)\-di-t-butylphenol), 4,4'-bis(2,6-di-t-butylphenol), 2,2'-methylenebis(4-methyl-6-t-butylphenol), 4,4'-thiobis(2-methyl-6-t-butylphenol), 2,2-thiodiethylenebis[3-(3,5-di-t-butyl-4-hydroxyphenyl)propionate], octyl 3-(3,5-di-t-butyl-4-hydroxyphenyl)propionate, octadecyl 3-(3,5-di-t-butyl-4-hydroxyphenyl)propionate, and octyl 3-(5-t-butyl-4-hydroxy-3-methylphenyl)propionate.

Examples of amine antioxidants are C₄₋₉ mixed alkyl diphenyl amines, p,p'-dioctyldiphenylamine, phenyl-α-naphthylamine, phenyl-β-naphthylamine, alkylated-α-naphthylamine, and alkylated-phenyl-α-naphthylamine.

Examples of molybdenum antioxidants are oxymolybdenum complexes of basic nitrogen compounds. Examples of preferred oxymolybdenum complexes of basic nitrogen compounds are oxymolybdenum complexes of succinimide and oxymolybdenum complexes of carbonamide. Oxymolybdenum complexes of basic nitrogen compounds can be produced using the following method, for instance. A molybdenum complex is produced by reacting an acidic molybdenum compound or salt thereof with a basic nitrogen compound, such as a succinimide, carbonamide, hydrocarbon monoamine, hydrocarbon polyamine, Mannich hydrochloric acid, phosphonamide, thiophosphonamide, phosphoric amide, dispersion-type viscosity index-improving agent (or a mixture thereof), while maintaining the reaction temperature at 120°C or lower.

Moreover, it is also possible to use a molybdenum-containing compound other than an oxymolybdenum complex of a basic nitrogen compound in place of the oxymolybdenum complex of the basic nitrogen compound, or in combination with the oxymolybdenum complex of a basic nitrogen compound. Examples of the combined molybdenum-containing compounds that can be used are sulfurized oxymolybdenum dithiocarbamates and sulfurized oxymolybdenum dithiophosphates.

The phenol antioxidant (particularly hindered phenol antioxidant), amine antioxidant (particularly diaryl amine antioxidant), and molybdenum antioxidant (particularly oxymolybdenum complex of basic nitrogen compound) can be used alone, or they can be used as an arbitrary combination with one another as desired. It is also possible to use these in combination with an oil-soluble antioxidant.

### Viscosity index-improving agent

The lubricating oil composition of the present invention further comprises a viscosity index-improving agent (component e) in an amount within a range of 0.5 to 20 mass%. Examples of viscosity index-improving agents are polymethacrylate viscosity index-improving agents such as polyalkylmethacrylate, and viscosity index-improving agents based on olefin copolymers, such as ethylene-propylene copolymer, styrene-butadiene copolymer, and polyisoprene. Of these viscosity index-improving agents, olefin copolymer viscosity index-improving agents have high thermal stability and are effective in terms of the object of the present invention. One having a shear stability index (SSI) of 30 or less (particularly 25 or less) is particularly preferable for the object of the present invention. Moreover, a dispersion-type viscosity index-improving agent or multifunctional viscosity index-improving agent that imparts dispersion performance to these polymer compounds is preferably used. These viscosity index-improving agents can be used alone, or a combination of any two or more viscosity index-improving agents can be used.

### Organic sulfur compound

Preferably the lubricating oil composition of the present invention further comprises an organic sulfur compound that is effective in terms of wear resistance and oxidation resistance. Examples of organic sulfur compounds having such a property are sulfurized olefins, sulfurized esters, sulfurized oils and fats, polysulfide compound, dimercaptothiadiazoles, dithiophosphoric acid esters, and dithiocarbamates.

### Other additives

The addition of an alkali metal borate hydrate to the lubricating oil composition of the present invention is effective in terms of high-temperature detergency and imparting a base value. The amount of alkali metal borate hydrate is 5 mass% or less, particularly 0.01 to 5 mass%. Alkali metal borate hydrates often have an ash component, sulfur component, and the like, but taking into consideration the properties of the lubricating oil composition of the present invention, an alkali metal borate hydrate can be effectively used by adjusting the amount added.

The lubricating oil composition of the present invention can also contain a small amount of various auxiliary additives. Examples of such auxiliary additives are zinc dithiocarbamate and methylene bis(dibutyl dithiocarbamate), oil-soluble copper compounds, and organic amide compounds (such as oleyl amide) that function as antioxidants or anti-wear agents. Moreover, it is possible to add compounds such as benzotriazole compounds and thiadiazole compounds that function as metal deactivators. It is possible to add polyoxyalkylene nonionic surfactants such as polyoxyethylene alkylphenyl ethers and copolymers of ethylene oxide and propylene oxide that function as anti-rust agents and demulsifiers. It is possible to add various amides, polyhydric alcohol aliphatic acid esters, or derivatives thereof that function as wear adjusters. Moreover, it is possible to add a variety of compounds that function as antifoaming agent and pour point depressants. Note that preferably these auxiliary additives are each used in an amount that is 3 mass% or less (particularly a range of 0.001 to 3 mass%) in terms of the lubricating oil composition.

### Examples

The present invention is further described by the following illustrative non-limiting working examples.

### [Examples 1 and 2, comparative examples, and reference examples]

### (1) Production of lubricating oil composition

The lubricating oil composition of the present invention (SAE viscosity grade: 5W20, high-temperature, high-shear viscosity: 2.9 mPa·s or higher) was produced (Examples 1 and 2) using the following base oil and additives (in the following amounts). Moreover, a lubricating oil composition having an SAE viscosity grade of 5W20 (high-temperature, high-shear viscosity of approximately 2.6 mPa·s) was produced as a comparative example and a lubricating oil composition having an SAE viscosity grade of 10W30 (high-temperature, high-shear viscosity of 2.9 mPa·s or higher) was produced as a reference example.

### (2) Base oil

Base oil1: Mixture (having viscosity index of 142, a kinematic viscosity at 100°C of 4.9 mm²/s, and NOACK evaporation loss of 10.1%) of mineral oil base oil a (having a viscosity index of 137, a kinematic viscosity at 100°C of 4.1 mm²/s, and a NOACK evaporation loss of 13.6%) obtained by hydrogenation and isomerization, fractionation, and then dewaxing using slack wax as the starting material and mineral oil base oil b (having a viscosity index of 148, a kinematic viscosity at 100°C of 6.6 mm²/s, and NOACK evaporation loss of 5.0%) obtained by hydrogenation and isomerization, fractionation, and then dewaxing using slack wax as the starting material, at a weight ratio of 60:40 (base oil a:base oil b).

Base oil 2: Hydrocracked mineral oil (having a viscosity index of 128, a kinematic viscosity at 100°C of 4.2 mm²/s, and NOACK evaporation loss of 14.2%)

Base oil 3: Mixture (having viscosity index of 115, kinematic viscosity at 100°C of 6.7 mm²/s, and NOACK evaporation loss of 10.8%) of hydrocracked mineral oil a (having a viscosity index of 122, a kinematic viscosity at 100°C of 5.6 mm²/s, and NOACK evaporation loss of 12.4%) and hydrocracked mineral oil b (having a viscosity index of 99, a kinematic viscosity at 100°C of 10.7 mm²/s, and NOACK evaporation loss of 6.0%), at a weight ratio of 73:27 (mineral oil a:mineral oil b)

Note: The amount of base oil that, together with the total amount of the following additives, brought the total to 100 mass%.

### (3) Additives

### [Nitrogen-containing ash-free dispersant]

1) Ash-free dispersant 1 (mass-average molecular weight: 5,100 (in terms of polystyrene by GPC analysis; same hereafter), nitrogen content: 1.95 mass%, boron content: 0.63 mass%, chlorine content: less than 5 ppm by mass; obtained by reacting a highly reactive polyisobutene having a number-average molecular weight of approximately 1,300 (at least approximately 50% of which had a methyl vinylidene structure) and maleic anhydride by thermal reaction, reacting the resulting polyisobutenyl succinic anhydride with a polyalkylene polyamine having an average number of nitrogen atoms of 6.5 (per one molecule) to obtain the bis-type of succinimide, and then reacting this bis-type of succinimide with boric acid)
   Amount added: 0.06 mass% (in terms of N)
2) ash-free dispersant 2 (mass-average molecular weight: 12,800, nitrogen content: 1.0 mass%, chlorine content: 30 ppm by mass; obtained by reacting a highly reactive polyisobutene having a number-average molecular weight of approximately 2,300 (at least approximately 50% of which had a methyl vinylidene structure) and maleic anhydride by thermal reaction, reacting the resulting polyisobutenyl succinic anhydride with a polyalkylene polyamine having an average number of nitrogen atoms of 6.5 (per one molecule) to obtain the bis-type of succinimide, and then reacting this bis-type of succinimide with ethylene carbonate)
   Amount added: 0.01 mass% (in terms of N)

### [Alkaline earth metal-containing detergent]

1) Perbasic calcium phenate (sulfurized phenate having C₁₂ branched alkyl groups, Ca: 9.6 mass%, S: 3.4 mass%, TBN: 264 mgKOH/g)
   Amount added: 0.15 mass% (in terms of Ca)
2) Perbasic calcium sulfonate (alkyl toluene sulfonate having C₂₀₋₂₄ alkyl groups, Ca: 16.0 mass%, S: 1.6 mass%, TBN: 425 mgKOH/g, degree of perbasic conversion: 19)
   Amount added: 0.07 mass% (in terms of Ca)
3) Low-basic calcium sulfonate (alkyl benzene sulfonate having C₁₄₋₂₄ alkyl groups, Ca: 2.4 mass%, S: 2.9 mass%, TBN: 17 mgKOH/g, degree of perbasic conversion: 0.34)
   Amount added: 0.01 mass% (in terms of Ca)

### [Zinc dithiophosphate]

Zinc di(secondary-alkyl) dithiophosphate (P: 7.2 mass%< Zn: 7.8 mass%, S: 14 mass%, produced derived from C₃₋₈ secondary alcohol)
Amount added: 0.06 mass% (in terms of P)
Zinc di(primary alkyl) dithiophosphate (P: 7.3 mass%, Zn: 8.4 mass%, S: 14 mass%, produced derived from C₈ primary alcohol)
Amount added: 0.03 mass% (in terms of P)

### [Antioxidant]

Dialkyl diphenyl amine (alkyl groups: mixture of C₄ and C₈, N: 4.6 mass)
Amount added: 0.45 mass%

### [Organic sulfur compound] (used in Example 2 only)

Sulfurized isobutylene (S: 42 mass%)
Amount added: 0.3 mass%

### [Viscosity index-improving agent]

Polymethacrylate viscosity index-improving agent (SSI = 18, mass-average molecular weight: 200,000) - used in examples 1 and 2 and comparative example
Amount added: 5.1 mass% (example 1), 5.0 mass% (example 2), 5.1 mass% (Comparative example)
Ethylene propylene copolymer viscosity index-improving agent (SSI = 24) - used in Reference example
   Amount added: 4.6 mass%

### [Pour point depressant]

Polymethacrylate pour point depressant: 0.3 mass%

### [Other additives]

Combination of small amounts each of additives such as anti-wear agent, anti-rust agent, defoaming agent, and the like
Amount added: 0.6 mass%

### Evaluation of lubricating oil composition

(1) Viscosity properties of lubricating oil composition (high-temperature, high-shear viscosity, kinematic viscosity (at 100°C and 40°C), viscosity index, cranking viscosity (at -25°C or -30°C) and pumping temperature (at -35°C) were determined under the conditions described below.
(2) Moreover, the NOACK evaporation loss (%) at 250°C of the lubricating oil composition was determined by ASTM D5800, method B.
(3) Furthermore, the Shell four spheres test was conducted as a test to evaluate wear resistance. According to the Shell four spheres test, sample oil was heated to 75°C and tests were performed for 60 minutes under a load of 40 kgf at 1,200 rotations per minute. The diameter of the abrasion scar left on the surface of the test spheres was determined.

Table 1 shows the properties of each of the lubricating oil compositions and the results of the Shell four spheres test of examples 1 and 2, the comparative example, and the reference example.

**Table 1**

| | **Example 1** | **Example 2** | **Comparative Example** | **Reference Example** |
|---|---|---|---|---|
| Viscosity grade | 5W20 | 5W20 | 5W20 | 10W30 |
| Base oil | Base oil 1 | Base oil 1 | Base oil 2 | Base oil 3 |
| High-temperature, high-shear viscosity | 2.93 | 2.91 | 2.62 | 3.15 |
| Kinematic viscosity (100°C) | 9.15 | 9.05 | 8.02 | 10.1 |
| Kinematic viscosity (40°C) | 44.1 | 43.7 | 36.3 | 65.7 |
| Viscosity index | 196 | 195 | 203 | 139 |
| Cranking viscosity | - | - | - | 5815 |
| -25°C | | | | |
| -30°C | 3630 | 3590 | 2800 | - |
| Pumping viscosity at -35°C | Passed | Passed | Passed | Passed^{∗} |
| NOACK evaporation loss (%) | 9.7 | 9.8 | 14.0 | 11.5 |
| Shell four spheres test | 0.47 | 0.47 | 0.54 | 0.48 |
| Average abrasion diameter (mm) | | | | |

| | | | | |
|---|---|---|---|---|
| Note: The high-temperature, high-shear viscosity is the viscosity at a shear speed of 10⁶s⁻¹ and temperature of 150°C (units mPa·s). The kinematic viscosity units are mm²/s and the cranking viscosity units are mPa·s. Moreover, a pumping viscosity that "passed" means that the pumping viscosity satisfied the regulation for pumping viscosity (at a determination temperature of -35°C) for SAE viscosity grade 5W20. However, the determination temperature was -30°C for pumping viscosity required by 10W30 and the "passed^{∗}" indicates that the determination passed the regulation for pumping viscosity at -30°C. | | | | |

The following are clear from the properties and results of evaluating each lubricating oil composition of examples 1 and 2, the comparative example, and the reference example shown in Table 1.
(1) The lubricating oil composition of examples 1 and 2 is an excellent fuel-efficient SAE grade 5W20 lubricating oil composition, but has virtually the same wear resistance as the SAE grade 10W30 lubricating oil composition of the reference example, which is of relatively inferior fuel efficiency.
(2) On the other hand, the lubricating oil composition of the comparative example has a high NOACK evaporation loss, low high-temperature, high-shear viscosity, and inferior wear resistance.

## Claims

1. A lubricating oil composition for automobile engine lubrication, which is a lubricating oil composition comprising a base oil and having an SAE viscosity grade of 5W20, wherein the viscosity index of the lubricating oil composition is within a range of 140 to 230, the high-shear viscosity at 150°C of the lubricating oil composition is 2.9 mPa·s or higher, and the NOACK evaporation loss of the lubricating oil composition is 13% or less, further comprising:
a) a nitrogen-containing ash-free dispersant at 0.01 to 0.3 mass% in terms of the nitrogen content,
b) an alkaline earth metal-containing detergent at 0.08 to 0.4 mass% in terms of alkaline earth metal content,
c) a phosphorus-containing anti-wear agent at 0.05 to 0.12 wt% in terms of phosphorus content,
d) an antioxidant selected from the group consisting of amine compounds, phenol compounds, and molybdenum compounds at 0.1 to 7 mass%,
e) a viscosity index-improving agent at 0.5 to 20 mass%, and further wherein
the amount of each additive component is the mass% in terms of the total amount of lubricating oil composition;
wherein the Noack evaporation loss is determined by ASTM D5800; and wherein the phrase "high-shear viscosity" refers to the measured value (shear viscosity) when the shear speed or shear rate is 10⁶s⁻¹, and
wherein the base oil is:
a base oil comprising as a base oil component at least 80 mass% of a mineral oil base oil having a kinematic viscosity at 100°C that is within a range of 2 to 9 mm²/s and a viscosity index of 133 to 160; or
a base oil having a viscosity index of 133 to 160 that is obtained by hydrogenation and isomerization of either a slack wax or a synthetic wax produced by the Fischer-Tropsch method and then distillation and dewaxing treatment.

2. The lubricating oil composition according to claim 1, wherein the base oil is a mineral oil having a kinematic viscosity at 100°C that is within a range of 2 to 9 mm²/s and a viscosity index of 133 to 160.

3. The lubricating oil composition according to claim 1, wherein the viscosity index-improving agent is a polymethacrylate polymer having a shear stability index of 30 or less.

4. The lubricating oil composition according to claim 1, which further comprises an organic sulfur compound as an additive component.

5. Use of the lubricating oil composition according to claim 1 for lubrication of a motorcycle four-cycle gasoline engine.

6. Use of the lubricating oil composition according to claim 1 for lubricating the engine of a diesel engine vehicle having an exhaust gas after-treatment device.

7. A method for lubricating a motorcycle four-cycle gasoline engine using the lubricating oil composition according to claim 1.

8. A method for lubricating an engine of a diesel engine vehicle having an exhaust gas after-treatment device using the lubricating oil composition according to claim 1.

## Patentansprüche

1. Schmierölzusammensetzung für Kraftwagenmotorschmierung, die eine Schmierölzusammensetzung ist, umfassend ein Grundöl mit einem SAE-Viskositätsgrad von 5W20, wobei der Viskositätsindex der Schmierölzusammensetzung innerhalb des Bereichs von 140 bis 230 ist, die Hochscher-Viskosität der Schmierölzusammensetzung bei 150°C 2,9 mPa·s oder höher ist, und der NOACK-Verdampfungsverlust der Schmierölzusammensetzung 13% oder weniger ist, zudem umfassend
a) ein stickstoffhaltiges, aschefreies Dispergiermittel mit 0,01 bis 0,3 Masse-% nach Stickstoffgehalt,
b) ein alkalierdmetallhaltiges Dispergiermittel mit 0,08 bis 0,4 Masse-% nach Alkalierdmetallgehalt,
c) ein phosphorhaltiges Antiabriebmittel mit 0,05 bis 0,12 Gew.-% nach Phosphorgehalt,
d) ein Antioxidans, ausgewählt aus der Gruppe Aminverbindungen, Phenolverbindungen und Molybdänverbindungen mit 0,1 bis 7 Masse-%,
e) ein Viskositätsindex-Verbesserungsmittel mit 0,5 bis 20 Masse-%, und zudem wobei
die Menge jedes Zusatzmittelbestandteils die Masse-% nach der Gesamtmenge Schmierölzusammensetzung ist;
wobei der NOACK-Verdampfungsverlust nach ASTM D5800 bestimmt wird; und
wobei der Begriff "Hochscher-Viskosität" sich auf den gemessenen Wert (Scherviskosität) bezieht, wenn die Schergeschwindigkeit oder Scherrate 10⁶ s⁻¹ ist, und
wobei das Grundöl ist
ein Grundöl, umfassend als Grundölbestandteil mindestens 80 Masse-% eines Mineralöl-Grundöls mit einer kinematischen Viskosität bei 100°C, die innerhalb eines Bereichs von 2 bis 9 mm²/s ist, und einem Viskositätsindex von 133 bis 160; oder
ein Grundöl mit einem Viskositätsindex von 133 bis 160, das erhalten wird durch Hydrogenisierung und Isomerierung, entweder eines Gatsches oder eines synthetischen Wachses, hergestellt durch das Fischer-Tropsch-Verfahren und dann Destillierung und Entwachsungsbehandlung.

2. Schmierölzusammensetzung gemäß Anspruch 1, wobei das Grundöl ein Mineralöl ist mit einer kinematischen Viskosität bei 100°C, die innerhalb eines Bereichs von 2 bis 9 mm²/s ist, und einem Viskositätsindex von 133 bis 160.

3. Schmierölzusammensetzung gemäß Anspruch 1, wobei das Viskositätsindex-Verbesserungsmittel ein Polymethacrylatpolymer ist mit einem Scherstabilitätsindex von 30 oder geringer.

4. Schmierölzusammensetzung gemäß Anspruch 1, die zudem eine organische Schwefelverbindung als Zusatzmittelbestandteil umfasst.

5. Verwendung der Schmierölzusammensetzung aus Anspruch 1 zur Schmierung eines Motorrad-Viertakt-Benzinmotors.

6. Verwendung der Schmierölzusammensetzung aus Anspruch 1 zur Schmierung des Motors eines Dieselmotorfahrzeugs mit einer Abgas-Nachbehandlungsvorrichtung.

7. Verfahren zum Schmieren eines Motorrad-Viertakt-Benzinmotors, das die Schmierölzusammensetzung aus Anspruch 1 verwendet.

8. Verfahren zum Schmieren eines Motors eines Dieselmotorfahrzeugs mit einer Abgas-Nachbehandlungsvorrichtung, das die Schmierölzusammensetzung aus Anspruch 1 verwendet.

## Revendications

1. Composition d'huile lubrifiante pour la lubrification d'un moteur automobile, qui est une composition d'huile lubrifiante comprenant une huile de base ayant un degré de viscosité SAE de 5W20, où l'indice de viscosité de la composition d'huile lubrifiante est dans l'intervalle de 140 à 230, la viscosité à cisaillement élevé à 150°C de la composition d'huile lubrifiante est 2,9 mPa·s ou plus, et la perte en évaporation NOACK de la composition d'huile lubrifiante est 13 % ou moins, comprenant en plus :
a) un dispersant libre en cendres et contenant de l'azote à 0,01 à 0,3 %-masse en termes de contenu en azote,
b) un détergent contenant un métal alcalino-terreux à 0,08 à 0,4 %-masse en termes de contenu en métal alcalino-terreux,
c) un agent anti-usure contenant du phosphore à 0,08 à 0,4 %-poids en termes de contenu en phosphore,
d) un antioxydant sélectionné parmi le groupe constitué en composés d'amine, composés de phénol, et composé de molybdène à 0,1 à 7 %-masse,
e) un agent d'amélioration d'indice de viscosité à 0,5 à 20 %-masse, et en plus où
la quantité de chaque composante d'additif est le 5-masse en termes du poids total de la composition d'huile lubrifiante ;
où la perte en évaporation NOACK est déterminée par ASTM D5800 ; et où l'expression « viscosité à cisaillement élevé » concerne à la valeur mesurée (viscosité de cisaillement) si la vitesse de cisaillement ou le degré de cisaillement est 10⁶ s⁻¹, et
où l'huile de base est :
une huile de base comprenant comme composante d'huile de base au moins 80 %-masse d'une huile de base à base d'une huile minérale ayant une viscosité cinématique à 100°C qui est dans l'intervalle de 2 à 9 mm²/s et un indice de viscosité de 133 à 160 ; ou
un huile da base ayant un indice de viscosité de à à 160 qui est obtenue par hydrogénation et isomérisation ou bien d'un gatsch ou d'une cire synthétique produite par le procédé Fischer-Tropsch, et ensuite une distillation et un traitement de décirage.

2. Composition d'huile lubrifiante selon la revendication 1, dans laquelle l'huile de base est une huile minérale ayant une viscosité cinématique à 100°C qui est dans l'intervalle de 2 à 9 mm²/s et un indice de viscosité de 133 à 160.

3. Composition d'huile lubrifiante selon la revendication 1, dans laquelle l'agent d'amélioration d'indice de viscosité est un polymère polyméthacrylate ayant un indice de stabilité de cisaillement de 30 ou moins.

4. Composition d'huile lubrifiante selon la revendication 1, qui comprend en plus un composé de soufre organique comme composante d'additif.

5. Utilisation de la composition d'huile lubrifiante de la revendication 1 pour lubrifier un moteur de motocyclette à quatre temps.

6. Utilisation de la composition d'huile lubrifiante de la revendication 1 pour lubrifier le moteur d'un véhicule diesel qui a un dispositif de traitement de gaz d'échappement.

7. Procédé pour lubrifier un moteur de motocyclette à quatre temps, utilisant la composition d'huile lubrifiante de la revendication 1.

8. Procédé pour lubrifier le moteur d'un véhicule diesel qui a un dispositif de traitement de gaz d'échappement, utilisant la composition d'huile lubrifiante de la revendication 1.
